

## UNITED STATES PATENT OFFICE

WALLACE C. BENNETT, OF HINGHAM, MASSACHUSETTS, ASSIGNOR TO BENNETT BOX CO., OF BOSTON, MASSACHUSETTS, A CORPORATION OF MASSACHUSETTS

## SHEET MATERIAL FOR SOFT BOXES FOR TOES AND METHOD OF MAKING SAME

No Drawing.

Application filed January 7, 1925. Serial No. 1,039.

This invention relates to improvements in sheet material, suitable for use for soft boxes for toes of shoes, and in method of making the same.

5 The making of a resilient soft box for a shoe presents a problem whose solution has not heretofore been known to the public so far as I am aware. Hence the best soft box shoes either omit the box material entirely, or else make a box which is flexible and thin in order to obtain the required softness, but which lacks the much desired quality of resilience and which has the additional disadvantage that it must be cemented to the adjacent sheets forming part 10 of the toe in order to form the integrated whole which is desirable. It is an object of the present invention to provide a soft box material in sheet form which when finished 15 will have the quality of resiliency in the toe and will to a satisfactory extent form an integrated unit with the lining and cap of the toe.

I have accomplished this purpose by providing 20 a composite sheet made of loosely matted pulp carried on a thin supporting fabric, of which cheese cloth is an example, the whole being treated with rubber latex or similar liquid.

25 The process of the invention by which this is accomplished is extremely simple. A sheet of repulped loosely matted and dried paper pulp, having thickness according to weight desired for the finished box, is laid 30 on the supporting fabric, and the two together are dipped into the rubber latex. When dry the product is a springy, flexible integrated sheet which can be dried into shape, skived if desired as is customary, 35 and lasted. Just before lasting it may be dipped into rubber latex, in which case, after lasting and drying, the box, lining and cap of the shoe will be found adhering firmly together, thus forming an integrated 40 toe which is soft and yet which is resiliently flexible.

An illustrative example of the practice of the invention will now be given. For the supporting fabric any suitably inexpensive 45 material, preferably cheese cloth, may be

used, the only requirement being that it should be strong enough to withstand the stresses of the lasting processes.

The term paper pulp as herein used is satisfied by the use of any lignocellulosic material composed of short somewhat stiff fibers, chiefly cellulose, prepared by treatment of wood or other ligneous matter from any kind of plant material, such as plant stems, stalks, or fibrous leaves, in a manner commercially known, or even that commercial product known as ground wood; but this pulp is to be used in a loosely matted condition, such as may be obtained from laying or depositing the raw pulped material 55 on a screen and letting it dry with little or no compression. Such a material is porous and absorbent, particularly so as compared with commercial paper pulp which has been subjected to high pressure and is only slowly absorbent; but it has a certain inherent stiffness, coupled with very little strength, especially as contrasted with the felt which is commonly used for toe boxes and which is a loosely matted material prepared from 60 long fibers, showing great flexibility and considerable strength. Such a pulp may be obtained by repulping commercial paper or pulp and depositing it in the desired 65 thickness.

A sheet of dry pulp of the above description, having a thickness which depends upon the desired thickness or weight of stiffening material to be used for the toe box, is placed on the cotton sheet and the two are 70 dipped together into the rubber latex. The latex may be the commercial material containing 25% to 40% of gum rubber, and preserved usually with ammonium hydroxide or a synthetic material prepared by re-colloiding ordinary rubber. The latex rapidly penetrates both the sheeting and the pulp, and these are then to be drained as soon as possible. The pulp lies on the sheeting as a very soft lining of fibers and 75 must be carefully handled. The excess of latex may be pressed out by rollers especially easily if covered with another layer of cloth. Having then been allowed to dry, either naturally or by the application of 80 85 90 95 100

heat, and either in loose form or preferably under sheet tension, the product is a flexible resilient integrated sheet. For the lasting the died portion or "disc" may be dipped in latex. This will produce a cementing of the resilient sheet material to the other sheet ingredients or elements of the toe box. Or if preferred any ordinary method of causing the sheet material to adhere to the lining of the shoe in the toe may be used. Moreover, the latex may be used by a vulcanizing method. In place of commercial latex any variety thereof containing vulcanizing material, or that has been vulcanized in the liquid form may be used, and the resulting material heated in the shoe to form a vulcanized toe.

The supporting sheet may be itself a composite product, having a quality of resiliency greater than that of cloth sheeting, prepared by any known or suitable method. Thus, the pulp may be laid on a cloth which has been made resilient by saturating it with anything which when cool and suitably treated gives it more body stiffness and elasticity than is natural to the cloth alone, thus producing a composite result which is more desirable for certain types of shoes. Any suitable method may be employed for softening such a stiffener, if necessary or desirable, for the lasting process.

It will be understood that the invention is not limited to the use of commercial rubber latex, for one may use any latex, natural or synthetic, that may serve the purpose, or any similar colloidal suspension of rubber particles resembling latex in its properties and action. And for the supporting sheet, the fabric need not be cheese cloth, which has been mentioned as being preferable, but may be a thin sheet or screening of any suitable textile or other material.

I claim as my invention,

45 1. In the manufacture of sheet material suitable for use in stiffeners for shoes and the like, the step of impregnating with a colloidal suspension of rubber a composite sheet comprising a supporting fabric and a superimposed body of loosely-matted short fibres derived from wood.

50 2. In the manufacture of stiffeners for shoes and the like, the steps of impregnating with a colloidal suspension of rubber a composite sheet comprising a supporting fabric and a superimposed body of loosely-matted short fibres derived from wood, drying the mass, and thereafter, for incorporating the same in a shoe or other article, developing thereon an adhesive surface.

55 3. A sheet material suitable for use as a stiffener for shoes and the like comprising a composite sheet having a fabric base and a superimposed body of loosely-matted short fibres derived from wood, said composite

sheet being impregnated with the residue of a colloidal suspension of rubber.

Signed at Boston, Massachusetts, this sixteenth day of December 1924.

WALLACE C. BENNETT.

70

75

80

85

90

95

100

105

110

115

120

125